

## UNITED STATES PATENT OFFICE

1,996,833

## MANUFACTURE OF METAL CARBONYLS

Leo Schlecht, Ludwigshafen-on-the-Rhine, and  
Emil Keunecke, Oppau, Germany, assignors to  
I. G. Farbenindustrie Aktiengesellschaft,  
Frankfort-on-the-Main, Germany

No Drawing. Application November 14, 1932,  
Serial No. 642,601. In Germany September 17,  
1928.

8 Claims. (Cl. 23—203)

The present invention relates to the production of metal carbonyls, more particularly from initial materials which contain the metal or metals, capable of reacting with carbon monoxide with the formation of metal carbonyls, in the form of a metal sulphide.

In order to convert initial materials of the said kind into metal carbonyls it has been customary prior to the present invention to make use of a three-stage process by first subjecting the initial material to a roasting process, whereby the sulphidic compounds are converted into oxides, then subjecting the material to a reduction treatment, whereby the metals capable of forming metal carbonyls are converted into the metallic state, and then acting on the reduced material with carbon monoxide.

It is the object of the present invention to simplify this process, so that initial materials of the said kind become readily and cheaply available for the production of metal carbonyls.

The process according to the present invention is based upon the surprising discovery that the gases and vapors formed during conversion of the initial material, by treatment with carbon monoxide, into the metallic state, such as carbon oxy-sulphide, hydrogen sulphide or carbon disulphide, do not interfere with the interaction of the metal or metals with the carbon monoxide for the formation of the metal carbonyl or carbonyls.

The process which we have developed out of this discovery consists, as has been set forth in our application for patent Ser. No. 387,791, filed August 22nd, 1929, of which this application is a continuation-in-part, in acting on an initial material of the aforesaid kind with carbon monoxide or a gas containing carbon monoxide under conditions, more particularly as regards the pressure and temperature and also the speed of the gas current, under which the formation of metal carbonyl takes place from initial material in the metallic state. Under such conditions the conversion of the initial material into the metallic state and the formation of the metal carbonyl or carbonyls proceed simultaneously in a satisfactory manner and at a sufficiently high speed, so that, instead of the old three-stage process, initial materials of the aforesaid kind can now be converted into metal carbonyls in only one stage, metal carbonyl being formed from the very start of the treatment.

We shall now proceed to explain more in detail the conditions under which the process according to the present invention is carried out.

Generally speaking, the pressure must be the higher, the higher the temperature. In this connection it must be borne in mind, that an equilibrium is set up in the gas in that on the one hand metal and carbon monoxide react with each other with the formation of carbonyl, and on the other hand the carbonyl tends to decompose to metal and carbon monoxide, in accordance with the formula



wherein Me is the metal capable of forming a metal carbonyl. Depending on the temperature and pressure, the one or the other of these reactions will predominate and thus the yield in carbonyl will be influenced. Regard must also be had to the equilibrium expressed by the following formula



In view of the aforesaid equilibria, attention must be given not only to the temperature and pressure, but also to the speed of the gas current and, in case a gas containing carbon monoxide is used, such as a mixture of carbon monoxide with nitrogen, hydrogen, carbon dioxide or methane, to the composition of the gas. All these influences are controlled by the law of mass action and are therefore readily determinable. It may be pointed out, however, that the speed of the gas current should usually be so high that the gaseous by-products of the reduction and also the metal carbonyl formed are carried away by the gas current. The temperature and pressure conditions, moreover, vary according to the nature of the metal, which is to be converted into the carbonyl. Such mutual interdependency of the temperature and pressure conditions is well known in the art from the production of metal carbonyls from metallic initial materials.

Generally speaking the temperature and pressure should be of the same order in the process according to the present invention as would be used in case the initial material were present in the metallic state. It is preferable to work at temperatures at which the carbon monoxide or the gases containing the same convert the metal compounds with a sufficient velocity into the metallic state, but the temperature must not be so high that the decomposition of the carbon monoxide becomes troublesome. By employing the carbon monoxide under pressure the permissible temperature is raised in consequence of the favorable state of the equilibrium of the reaction between the metals and the carbon monoxide,

and it is preferable to choose the pressure and the temperature so high that the greatest possible quantity of carbonyl is formed. In order to keep the temperature as low as possible, in some cases, for example when using difficultly reacting materials, other substances which facilitate the conversion into the metallic state, as for example copper, lime or caustic alkalies, may be added to the material which forms the carbonyl.

Generally speaking temperatures between about 200° and about 450° C. and pressures of 20 atmospheres and more are suitable for the process in accordance with the present invention.

The mutual interdependency of the temperature and pressure conditions will now be explained further by reference to some specific examples, to which, however, the invention is not restricted.

#### Example 1

Nickel sulphide precipitated by means of ammonium sulphide from a nickel salt solution is treated with streaming carbon monoxide under a pressure of 200 atmospheres and at 200° C. In the course of 2 hours 90 per cent of the nickel is converted into nickel carbonyl.

The carbon oxysulphide formed as a by-product can be recovered as such or it may be destroyed for example by means of alkaline agents whereby carbon monoxide is regenerated. The spent alkaline agents may then be further treated for the production of elementary sulphur, or they may be treated for the production of hydrogen sulphide which can then be used for precipitating metals from the solutions obtained in the leaching of ores. The sulphides obtained may then advantageously be used for the production of metal carbonyls. At 200° C. and at a pressure of 200 atmospheres practically exclusively nickel sulphide is converted into nickel carbonyl by carbon monoxide. Under the said conditions the sulphides of other carbonyl-forming metals react only very difficultly with carbon monoxide. For the conversion of these sulphides higher temperatures or higher pressures or both must be used. In this way not only separation of the carbonyl-forming metals from the metals not capable of forming carbonyls is effected, but also the carbonyl-forming metals are separated from each other and especially the nickel is separated from iron and cobalt. Since the hydrogen sulphide can be easily regenerated in this manner of working and can be used again for the precipitation, the process is very suitable for the treatment of large amounts of leaching solutions and especially such as are so low in metals that their treatment was not economical hitherto.

#### Example 2

Precipitated iron sulphide is acted upon with a current of carbon monoxide at between 200° and 300° C. and under a pressure of 1000 atmospheres. From 70 to 80 per cent of the iron present is converted into iron carbonyl.

#### Example 3

Carbon monoxide is allowed to act at between 200° and 250° C. and under a pressure of 200 atmospheres on a mixture of precipitated iron sulphide and precipitated nickel sulphide. 95 per cent of the nickel present is converted into nickel carbonyl which is contaminated with only small amounts of iron carbonyl.

The solid residue is roasted in a current of air, then reduced with hydrogen at 480° C. and then treated with carbon monoxide under the conditions specified above. From 80 to 90 per cent of the iron is converted into iron carbonyl.

Generally speaking, it is advisable to work at between 150° and 275° C. and under a pressure of at least 50 or 100 atmospheres for the production of nickel carbonyl and at between 220° and 300° C. and under a pressure of at least 300 atmospheres for the production of iron carbonyl.

It will be seen from the foregoing that the process according to the present invention is carried out under the same conditions under which the treatment with carbon monoxide would be effected if the metal or metals capable of forming metal carbonyls were initially present in the metallic state. The same is true with regard to the apparatus which are suitable for carrying out the process according to the present invention.

In case several metal carbonyls are formed simultaneously, they may be separated from each other in any suitable manner, as for example by the methods of fractionation described and claimed in the copending application for patent, Ser. No. 637,200, filed October 10th, 1932, by Carl Müller and ourselves.

In the case of initial materials containing two or more metals capable of forming metal carbonyls, it may be advantageous first to convert mainly one metal sulphide into the corresponding metal carbonyl by the process according to the present invention, and then to subject the material under treatment to the old three-stage process by roasting, reduction and subsequent treatment with carbon monoxide for the recovery of the remaining metal or metals capable of forming a metal carbonyl. This method of working is illustrated by Example 3 given above.

When working with streaming carbon monoxide and when employing the excess of gas in a circular course, it is advantageous to remove from the gas under circulation, either wholly or partly, the by-products formed by the conversion of the initial materials into the metallic state, such as carbon oxysulphide, carbon disulphide or hydrogen sulphide, and other impurities; for example, carbon oxysulphide may be removed when working under elevated pressure, by scrubbing the gas with aqueous or alcoholic caustic alkali solutions under pressure, after the metal carbonyl has been separated from the gas.

The process according to the present invention is applicable to the treatment not only of metal sulphide or materials containing the same, but also of such compounds or mixtures of compounds as are capable of being converted, under the conditions of the treatment with carbon monoxide, into the metal sulphides; as examples of such compounds or mixtures of compounds may be mentioned moist mixtures of alkali metal sulphides with metal sulphates or metal chlorides or other metal salts. Suitable initial materials of the said kind are for example sulphidic ores or metallurgical intermediate or waste products such as those resulting from precipitation processes. All such initial materials are to be regarded as equivalents for the purposes of the present invention and are therefore comprised in the following claims by the term "material comprising a sulphidic compound".

What we claim is:—

1. The process of producing metal carbonyls which comprises acting with carbon monoxide on a material comprising a sulphidic compound of at

least one metal capable of forming a metal carbonyl, under conditions of temperature and pressure, under which formation of a metal carbonyl would take place if the metal of said sulphidic compound were present in the metallic state.

2. The process of producing metal carbonyls which comprises acting with carbon monoxide on a material comprising a sulphidic compound of at least one metal capable of forming a metal carbonyl at between about 150° and about 450° C. and under a pressure of at least 20 atmospheres.

3. The process of producing nickel carbonyl which comprises acting with carbon monoxide on a material comprising a sulphidic compound of nickel at between about 150° and about 450° C. and under a pressure of at least 20 atmospheres.

4. The process of producing nickel carbonyl which comprises acting with carbon monoxide on a material comprising a sulphidic compound of nickel at between 150° and 275° C. and under a pressure of at least 50 atmospheres.

5. The process of producing nickel carbonyl

which comprises acting with carbon monoxide on a material comprising a sulphidic compound of nickel at 200° C. and under a pressure of 200 atmospheres.

6. The process of producing iron carbonyl which comprises acting with carbon monoxide on a material comprising a sulphidic compound of iron at between about 150° and about 450° C. and under a pressure of at least 20 atmospheres.

7. The process of producing iron carbonyl which comprises acting with carbon monoxide on a material comprising a sulphidic compound of iron at between 220° and 300° C. and under a pressure of at least 300 atmospheres.

8. The process of producing iron carbonyl which comprises acting with carbon monoxide on a material comprising a sulphidic compound of iron at between 220° and 300° C. and under a pressure of 1000 atmospheres.

LEO SCHLECHT.  
EMIL KEUNECKE.